

March 5, 1946.

F. R. HENSEL

2,396,100

ELECTRIC CONTACT

Filed June 30, 1943



ELECTRIC CONTACT  
FORMED OF GOLD  
BASE ALLOY  
CONTAINING LEAD  
OR THALLIUM

Fig. 1



Fig. 2

INVENTOR.  
BY FRANZ R. HENSEL  
Robbin & Carlson  
ATTORNEYS

## UNITED STATES PATENT OFFICE

2,396,100

## ELECTRIC CONTACT

Franz R. Hensel, Indianapolis, Ind., assignor to  
 P. R. Mallory & Co., Inc., Indianapolis, Ind., a  
 corporation of Delaware

Application June 30, 1943, Serial No. 492,917

3 Claims. (Cl. 200—166)

This invention relates to electric contacts.

An object of the invention is to improve electric contact compositions.

Other objects of the invention will be apparent from the description and claims.

Figure 1 is a plan view of a contact embodying this invention; and

Figure 2 is a side elevation of the structure of Figure 1.

The present invention contemplates an electric contact formed of a gold base alloy containing lead or thallium.

The contact alloys may contain:

|                                     | Per cent<br>by weight |
|-------------------------------------|-----------------------|
| Lead, thallium or lead and thallium | 0.1 to 15             |
| Gold or gold base alloys            | Balance               |

The gold used may be either pure gold or one of the carat golds. These consist of gold-base alloys containing additions of silver, copper or other metals such as nickel, zinc, palladium, platinum or manganese. A table of carat golds is given in Metals Handbook (American Society for Metals, Cleveland, Ohio) 1939 edition, page 1507. It is contemplated that silver or copper may be present in the metal composition from traces to 20%, and hence are sometimes present in proportions still higher than would be present if carat golds were used in making the compositions.

The preferred contact materials for most uses contain:

|                                     | Per cent<br>by weight |
|-------------------------------------|-----------------------|
| Lead, thallium or lead and thallium | 0.5 to 5              |
| Gold                                | Balance               |

Examples of suitable specific contact materials are:

| (a)  | Per cent |
|------|----------|
| Lead | 1        |
| Gold | 99       |

| (b)      | Per cent |
|----------|----------|
| Thallium | 2.5      |
| Gold     | 97.5     |

| (c)      | Per cent |
|----------|----------|
| Lead     | 1        |
| Thallium | 1        |
| Gold     | 98       |

| (d)    | Per cent |
|--------|----------|
| Lead   | 3        |
| Silver | 15       |
| Gold   | 82       |

The contact alloys can be made by conventional alloying methods, as by melting the ingredients together.

The alloys can also be made by powder metallurgical methods, consisting in mixing the powders, pressing same and then sintering them at a temperature where the ingredients diffuse into each other. In certain cases, it may be advisable to mix oxide powders of the lead and thallium with the gold base material and then carry out the sintering in a reducing atmosphere. In certain cases it may be advisable to retain a certain percentage of oxides in the alloy and for such applications the sintering may be carried out in a neutral or oxidizing atmosphere.

Contacts of the present invention find application in various electric devices, such as relays, voltage regulators, meters, gauges, telephone relays, thermostatic applications, sliding contacts and brush applications where certain anti-friction properties are required.

These contacts have the advantages of tarnish resistance and thereby low contact resistance. They can be operated at low pressures both in D. C. and A. C. circuits. The presence of lead and thallium in the percentages covered by the present invention, provides a finely distributed phase which, during the operation of the contacts, tends to form a non-wetting oxide. The percentages of this oxide are so calculated that they will hardly affect the contact resistance but will greatly decrease the sticking tendencies of the contacts. Due to the fact that the gold-thallium and gold-lead systems are eutectic compositions, the metals lead and thallium are present in elementary form or metal compounds. The distribution, therefore, of the non-wetting constituent is microscopically fine. During the operation of the contacts, and particularly during the arc stage, a slight oxidation of these microscopical particles prevents welding of the contacts because gold areas which might be momentarily fused will have no chance to flow together, thereby forming a large enough molten pool to cause sticking.

While specific embodiments of the invention have been described, it is intended to cover the invention broadly within the spirit and scope of the appended claims.

What is claimed is:

- An electric contact formed of a gold base alloy containing 0.1 to 15% of metal selected from the group consisting of lead and thallium.
- An electric contact composed of 0.1 to 15% of metal selected from the group consisting of lead and thallium, balance substantially all gold, said contact being characterized by low contact resistance and the presence of a finely distributed phase formed predominantly of the lead or thallium capable of decreasing the sticking tendency of the contact.
- An electric contact composed of 0.5 to 5% of metal selected from the group consisting of lead and thallium, balance gold.

FRANZ R. HENSEL.